

# UNITED STATES PATENT OFFICE.

GUILLIAM H. CLAMER AND JOSEPH G. HENDRICKSON, OF PHILADELPHIA, PENNSYLVANIA, ASSIGNORS TO THE AJAX METAL COMPANY, OF SAME PLACE.

## ALLOY.

SPECIFICATION forming part of Letters Patent No. 655,392, dated August 7, 1900.

Application filed March 13, 1900. Serial No. 8,493. (No specimens.)

*To all whom it may concern:*

Be it known that we, GUILLIAM H. CLAMER and JOSEPH G. HENDRICKSON, citizens of the United States, residing at the city of Philadelphia, in the county of Philadelphia and State of Pennsylvania, have invented a certain new and useful Alloy, of which the following is a specification.

The object of the present invention is to provide for the convenient addition of tin, lead, and nickel to copper or copper compositions, so as to make so-called "composition castings." It may be remarked that the addition of nickel to such castings brings about a homogeneous distribution of lead and also prevents segregation. Lead is valuable in these castings, because it makes them solid and easily workable.

An alloy embodying the invention consists of lead, tin, and nickel in substantially the following proportions: lead, forty-five; tin, forty-five, and nickel, ten, and it is used by melting it along with copper or copper-bearing material in the proportion of, for example, one part of alloy to ten parts of copper, more or less.

An alloy embodying the present invention

may be made as follows: Nickel is added to tin. However, the nickel is readily soluble in melted tin, so that the amount which may be added depends only on temperature and time given for the solution. The temperature required is only a red heat and is far below the melting-point of nickel. After the tin has absorbed the requisite amount of nickel the lead is added to form the finished product. It is then cast in suitable molds in bars of convenient size.

Having thus described the nature and objects of our invention, what we claim as new, and desire to secure by Letters Patent, is—

A composition for admixture to copper castings which consists of an alloy of lead, tin and nickel, substantially as described.

In testimony whereof we have hereunto signed our names in the presence of two witnesses.

G. H. CLAMER.

J. G. HENDRICKSON.

Witnesses:

W. R. WOOTERS,  
LOUIS P. DOERING.